# EUROPEAN PATENT SPECIFICATION

(11) **EP 2 031 079 B1**
(45) Date of publication and mention of the grant of the patent: **13.01.2021**
(21) Application number: 06767202.2
(22) Date of filing: 16.06.2006
(51) Int. Cl.: C21D 9/46, C21D 8/12, C22C 38/00, C22C 38/60, H01F 1/147, H01F 1/16

(54) **HIGH-STRENGTH ELECTROMAGNETIC STEEL SHEET AND PROCESS FOR PRODUCING THE SAME**
HOCHFESTE ELEKTROMAGNETISCHE STAHLPLATTE UND HERSTELLUNGSVERFAHREN DAFÜR
TÔLE EN ACIER ÉLECTROMAGNÉTIQUE DE RÉSISTANCE ÉLÉVÉÉ ET SON PROCÉDÉ DE FABRICATION

(43) Date of publication of application: 04.03.2009
(73) Proprietor: Nippon Steel Corporation, Tokyo (JP)
(72) Inventor: MURAKAMI, Hidekuni, Kitakyushu-shi Fukuoka 804-8501 (JP)
(74) Representative: Vossius & Partner Patentanwälte Rechtsanwälte mbB
(86) International application number: PCT/JP2006/312552
(87) International publication number: WO 2007/144964

(56) References cited:
- WO-A1-2005/033349
- JP-A- H09 125 148
- JP-A- 2005 113 185
- JP-A- 2006 009 048
- JP-A- 2006 070 348
- JP-A- 2006 169 611
- JP-A- 2006 169 615

## Description

### TECHNICAL FIELD

The present invention relates to a method for producing a high strength electrical steel sheet, more particularly high strength nonoriented electrical steel sheet.

### BACKGROUND ART

In the past, for the material for rotors, laminated electrical steel sheet has been used, but recently in applications where high speed rotation and larger rotor size are demanded, the possibility has arisen of the centrifugal force applied to the rotors exceeding the strength of the electrical steel sheets. Further, there are also many motors of structures assembling magnets into the rotors. Even if the rotational speed is not that high, the load applied to the rotor material itself during rotation of the rotor becomes large. In terms of the fatigue strength as well, the strength of the material is becoming a problem in increasing cases.

Further, electromagnetic switches become worn at the contact surfaces along with use, so a magnetic material superior in not only the electromagnetic properties, but also the wear resistance is desired.

To deal with these needs, recently high strength nonoriented electrical steel sheet has been studied and several proposals have been made. For example, Japanese Patent Publication (A) No. 1-162748 and Japanese Patent Publication (A) No. 61-84360 propose using as a material a slab raised in Si content and further containing one or more of Mn, Ni, Mo, Cr, and other solid solution strengthening ingredients, but sheet breakage is liable to frequently occur at the time of rolling. This causes a drop in productivity and a drop in yield, so there is room for improvement. Further, since Ni, Mo, and Cr are included in large amounts, the material becomes extremely expensive. Japanese Patent Publication (A) No. 2005-113185 and Japanese Patent Publication (A) No. 2006-070348 disclose nonoriented electrical steel sheet in which worked structures are left to obtain strength, while Japanese Patent Publication (A) No. 2006-009048 and Japanese Patent Publication (A) No. 2006-070296 disclose nonoriented electrical steel sheet in which additionally Nb etc. are incorporated in solid solution to suppress recrystallization. However, these do not pay particular attention to the crystal grain size before formation of the worked structures, so there is the problem that a stable iron loss cannot be obtained.

Further, technology relating to electrical steel sheet including a large amount of Cu is disclosed in Japanese Patent Publication (A) No. 2004-84053 and Japanese Patent Publication (A) No. 2004-99926, but due to the Cu phase precipitated in the steel, the reduction of the eddy current loss cannot be said to be sufficient. There is room for improvement for applications where the high frequency properties become a problem.

### DISCLOSURE OF THE INVENTION

As explained above, various proposals have been made regarding high strength electrical steel sheet, but the fact is that industrially stable production using ordinary electrical steel sheet production facilities while securing the necessary magnetic properties has not yet been reached. The inventors previously filed an application for high strength electrical steel sheet leaving worked structures in the steel sheet in Japanese Patent Application No. 2003-347084.

This technology was made based on the fact that even if leaving worked structures in the crystal structure, the magnetic properties do not deteriorate that much, that if considering the effect on raising the strength, the result is in no way inferior to a material strengthened by the conventional solid solution elements or precipitates and, not only that, if considering the productivity and the in-plane anisotropy of the magnetic properties, in particular the magnetic flux density, this is extremely useful technology. However, the clear metallurgy has not been established for how to improve the balance of magnetic properties and mechanical properties for electrical steel sheet having worked structures. On this point, no proof has been obtained that this technology is optimal.

The inventors engaged in detailed experiments to illuminate this point, in particular regarding the effects of the structure before rolling, and discovered that in electrical steel sheet having worked structures, there is an optimum region for achieving both good magnetic properties and mechanical properties and therefore succeeded in setting an industrially optimum range considering further productivity, in particular the processability of steel strips.

The present invention has as its object the stable on-line production of high strength nonoriented electrical steel sheet having a high strength of a tensile strength (TS) of for example 500 MPa or more and wear resistance and provided with superior magnetic properties of magnetic flux density (B50), iron loss, etc. particularly when used under a high frequency magnetic field, such as a motor rotating at a high speed, without, for example, being changed in cold rollability, annealing work efficiency, etc. from ordinary electrical steel sheet. The present invention was made to solve the above problem and is defined in the claims.

### BRIEF DESCRIPTION OF THE DRAWINGS

FIG. 1 is a view showing the strength-iron loss balance dependent on the grain size before working.

### BEST MODE FOR CARRYING OUT THE INVENTION

The inventors engaged in various experiments and studies to achieve this object. That is, the present invention provides a steel sheet containing C: 0.060% or less, Si: 0.2 to 3.2%, Mn: 0.05 to 3.0%, P: 0.30% or less, S or Se: 0.040% or less, Al: 2.50% or less, and N: or 0.040% less and optionally further containing, in accordance with need, one or both of Cu: 0.001 to 30.0% and Nb: 0.03 to 8.0%, wherein (1) the steel sheet structure is given worked structures and dislocation strengthening is used to increase the strength, (2) the crystal structure is coarsened right before forming the worked structures to finally remain in the steel sheet, and (3) the above crystal structure is limited from the viewpoint of the amount of Si to improve the processability so as to provide electrical steel sheet in which worked structures are left and formed wherein the balance of strength and magnetic properties is improved at a high productivity without causing trouble in work efficiency etc.

### [Composition of Ingredients]

First, the composition of ingredients of the high strength electrical steel sheet according to the present invention will be explained.

C causes deterioration of the magnetic properties, so the content is made 0.060% or less. On the other hand, it effectively acts to improve the texture and has the effect of suppressing the development of the {111} orientation not preferable to the magnetic properties and promoting the development of the preferable {110}, {100}, {114}, and other orientations. Further, from the viewpoints of increasing the strength, in particular raising the yield stress, improving the warm strength and creep strength, and improving the warm fatigue characteristics, in the case of Nb-containing steel, due to having the effect of retarding the recrystallization by NbC, the content is preferably 0.0031 to 0.0301%, more preferably 0.0051 to 0.0221%, more preferably 0.0071 to 0.0181%, more preferably 0.0081 to 0.0151%.

When the above such effect by C is particularly stressed or when the demands on the magnetic aging are particularly extremely tough, up to the slab stage, from the viewpoint of the deoxidizing efficiency, it is possible to include higher C and reduce the C by decarburizing annealing after formation of the coil. When reducing the content to 0.010% or so or less, from the viewpoint of the production cost, it is advantageous to reduce the amount of C by degassing facilities at the molten steel stage. In particular, if made 0.0020% or less, there is a remarkable effect of reduction of the iron loss. In the invention steel not requiring carbides or other nonmetallic precipitates for increasing the strength, even 0.0015% or less enables an increase in strength while further even 0.0010% or less enables a sufficient increase in strength.

Si increases the inherent resistance of the steel to reduce the eddy current and reduce the iron loss and raises the tensile strength, but if the amount added is less than 0.2%, that effect is small. The content is preferably 1.0% or more, more preferably 1.5% or more, more preferably 2.0% or more, more preferably 2.5% or more. In general, when used under a high frequency magnetic field, the loss due to the eddy current becomes larger, but even in the invention steel containing worked structures, to suppress this eddy current loss, it is effective to raise the Si content. However, if over 6.5%, the steel is made remarkably brittle. To further reduce the magnetic flux density of the product, the content is made 6.5% or less, preferably 4.0% or less. The optimum range of the amount of Si, as explained above, is determined considering also the crystal structure right before the formation of the worked structures to finally remain inside the steel sheet - an important factor of the present invention.
Since according to the present invention the content of Si is 3.2% or less, it no longer becomes necessary to consider embrittlement much at all. Further, the content may be made less than 2.0%, less than 1.5%, and less than 1.0%.

Note that in the case of utilization of the later explained solid solution Cu, Si is effective for suppressing the formation of the austenite phase at a high temperature, stabilizing the ferrite phase even at a high temperature, and making the effect of reduction of the eddy current loss by the solid solution Cu remarkable, but with an amount of addition of less than 1.5%, this effect is small. In particular, in low Si steel, the effect of reduction of the eddy current loss by the solid solution C tends to become weaker, so preferably 2.1% or more, more preferably 2.6% or more Si is contained.

Mn may be positively added to raise the strength of the steel, but is not particularly required for the purpose in the steel of the present invention utilizing the worked structures as the main means for increasing the strength. This is added for the purpose of raising the inherent resistance or enlarging the sulfides and promoting crystal grain growth and thereby reducing the eddy current loss and reducing the iron loss, but excessive addition not only causes a drop in the magnetic flux density, but also promotes the formation of the austenite phase at a high temperature, so the content is made 0.05 to 3.0%, preferably 0.5% to 2.5%, preferably 0.5% to 2.0%, more preferably 0.8% to 1.2%.

P is an element with a remarkable effect in raising the tensile strength and contributes to stabilization of the ferrite phase at a high temperature, but in the same way as the above Mn, in the present invention steel, addition is not really required. If over 0.3%, the embrittlement becomes great and industrial scale hot rolling, cold rolling, and other processing become difficult, so the upper limit is made 0.30%. The amount is preferably 0.20% or less, more preferably 0.15% or less.

S easily bonds with the Cu added in accordance with need in the invention steels, has an effect on the behavior in formation of a metal phase mainly comprised of Cu important for the purpose of addition of Cu, and sometimes causes reduction of the strengthening efficiency, so caution is required when including it in a large amount. Further, depending on the heat treatment conditions, it is possible to positively form fine Cu sulfides and promote higher strength. The produced sulfides sometime cause deterioration of the magnetic properties, in particular the iron loss. In particular, when the control value of the iron loss is strict, the content of S is preferably low and is limited to 0.040% or less. The content is preferably 0.020% or less, more preferably 0.010% or less. Se also has substantially the same effect as S.

Al is usually added as a deoxidizing agent, but it is possible to keep down the addition of Al and use Si for deoxidation. In Si deoxidized steel with an amount of Al of 0.005% or so or less, AlN is not produced, so this also has the effect of reducing the iron loss. Conversely, it is also possible to positively add it to promote the coarsening of the AlN and use the increase in inherent resistance to reduce the iron loss, but if over 2.50%, the embrittlement becomes a problem, so the content is made 2.50% to less than 2.0% or less than 1.8%.

Note that when utilizing solid solution Cu as the strengthening element, from the viewpoints of deoxidation and formation of nitrides as well, solid solution Al is positively added to stabilize the ferrite phase at a high temperature and suppress the eddy current loss due to the increase in the electrical resistance. Further, this also has the effect of promoting the remarkable effect of reduction of the eddy current loss by the solid solution Cu. In the same way as Si, this is preferably positively added. The content is preferably 0.3% or more, more preferably 0.6% or more, more preferably 1.1% or more, more preferably 1.6% or more, more preferably 2.1% or more. However, if over 2.50%, the castability and embrittlement become problems, so the content is made 2.50% or less.

N, like C, causes the magnetic properties to deteriorate, so the content is made 0.040% or less. In Si deoxidized steel with an Al content of 0.005% or so or less, like C, it is an element having the effects of increasing the strength, in particularly raising the yield stress, improving the warm strength and creep strength, and improving the warm fatigue characteristics and, in the case of Nb-containing steel, retarding recrystallization by NbN, and also effective from the viewpoint of improving the texture. From this viewpoint, the content is preferably 0.0031 to 0.0301%, more preferably 0.0051 to 0.0221%, more preferably 0.0061 to 0.0200%, more preferably 0.0071 to 0.0181%, more preferably 0.0081 to 0.0151%. When Al is 0.010% or so or more, inclusion of a large amount of N enables the formation of fine AlN and an enhancement of the recrystallization retardation effect, but the efficiency of retarding recrystallization is poor and the detrimental effect on the magnetic properties is also relatively large, so there is really no need for addition. In Al deoxidized steel, N should be 0.0040% or less. When no rise in strength due to nitrides or recrystallization retardation effect is expected, N is preferably as low as possible. If made 0.0027% or less, the effect of suppression of magnetic aging or deterioration of characteristics by AlN in Al-containing steel is remarkable. The content is more preferably 0.0022%, more preferably 0.0015% or less. Cu is included in the present invention in accordance with need; if added its content is 0.001 to 30.0%.Cu, if present as solid solution Cu, has the effect of raising the recrystallization degree of steel sheet and retarding recrystallization of the steel sheet. In the work strengthening of the present invention, such an effect appears from 0.001% or so. Depending on the amount of impurities, it is possible to obtain this effect by Cu even without positively adding Cu, but preferably Cu is made 0.002% or more, 0.003% or more, 0.005% or more, 0.007% or more, 0.01% or more, 0.02% or more, 0.03% or more, 0.04% or more, 0.05% or more, further 0.1% or more, 0.5% or more, 1.0% or more, or 2.0% or more. If so, the effect appears more. If the content of Cu is low, the recrystallization retardation effect becomes small, the heat treatment conditions for obtaining the recrystallization retardation effect are limited to a narrow range, and the freedom of management of the production conditions and adjustment of production becomes smaller in some cases. On the other hand, if the content of Cu is excessively high, the effect on the magnetic properties becomes large and in particular the rise in the iron loss becomes remarkable in some cases, so the upper limit from this viewpoint is 8.0%, particularly preferably 5.5% or less. From the viewpoint of the cost of addition, the content may be made less than 0.1%, further less than 0.01.

In conventional steel, in such a low Cu region, almost no effect of Cu is seen, but in the present invention steel, even with such a small amount of Cu, a good effect appears on the improvement of the yield strength-iron loss balance. This mechanism is not clear, but is believed to be as follows. The high density dislocations present in steel such as the invention steels can be said to be necessary for securing strength and at the very least raise the iron loss. The rise in the yield strength is related to the interaction between the dislocations remaining in the steel and the dislocations newly introduced when deforming the steel sheet and the ease of activity of the dislocations remaining in the steel. The stronger the interactions or the harder the activity of existing dislocations, the more the yield strength rises. On the other hand, the iron loss is related to the interaction between dislocations remaining in the steel and the domain walls moving at the time of application of a magnetic field. The smaller this interaction, the more the rise in iron loss is suppressed. As a result, the interaction with the dislocations becomes greater (or the remaining dislocations themselves become less active). If a large number of dislocations with small interaction with the domain walls are left, the yield strength-iron loss balance is improved. The magnitude of the interaction is basically considered to be related to the stress fields around the dislocations (strain of crystal lattice). It is believed that a small amount of Cu segregates around the remaining dislocations and forms optimum stress fields for the improvement of the yield strength-iron loss balance, preferable dislocations are selectively proliferated in the process of forming the remaining dislocations, or preferable dislocations are made to selectively remain in the annealing process. At what stage the effect of the small amount of Cu is exhibited is not clear, but the change in the stress field due to the difference in atomic radius between the Cu and Fe may be explained as one factor.

On the other hand, the inventors already filed an application for technology forming a metal phase mainly comprised of Cu in electrical steel sheet (hereinafter in the Description described as a "Cu metal phase") to try to achieve higher strength. When it comes to the Cu metal phase, combination with this application does not detract from the effects of the present invention in any way. While not particularly limited to this, the size of the Cu metal phase or Nb precipitates present in the invention steel is preferably 0.20 µm or less. If exceeding this, the efficiency of recrystallization retardation falls, a large amount of metal phase becomes necessary, and also the detrimental effect on the magnetic properties easily becomes larger. Further, while not particularly limited to this, the numerical density of the Cu metal phase or Nb precipitates is limited to the range able to be handled in view of the relationship with the Cu, Nb, or C content and the size of the precipitated phase. 20/µm³ or more or so is desirable. This effect is achieved in the above range of concentration of Cu.

Further, when utilizing solid solution Cu as the strengthening element, the range of Cu for achieving good high frequency properties may be made 2.0 to 30.0%. If the content of Cu is low, the eddy current loss reduction effect becomes small. On the other hand, if the content of Cu is too high, suppressing production of the metal phases mainly comprised of Cu becomes difficult and the eddy current loss reduction effect becomes smaller. Not only this, when forming relatively coarse Cu metal phases, the hysteresis loss is liable to be greatly increased and cracks and defects in the steel sheet at the time of rolling are liable to become worse.

Therefore, the content of Cu in this case is preferably 2.1% or more, more preferably 2.6% or more, more preferably 3.1% or more, more preferably 3.6% or more, more preferably 4.1% or more, more preferably 4.6% or more. The upper limit, considering also the cost of addition of Cu itself and the cost of addition of Ni added for the purpose of suppressing surface defects at the time of hot rolling due to Cu (Cu defects), is preferably 20.0%, more preferably 15.0%, more preferably 12.0%, more preferably 10.0%. Note that if the Cu added in the high Si steel in such a case is in the state of a solid solution, it will not cause embrittlement of the steel or deterioration of the cold rollability like Si or Al. Rather, it will have a preferable action in suppressing embrittlement due to Si etc. Further, it does not cause a great deterioration in the magnetic flux density like the later mentioned Cr and is of little harm even if included in a relatively large amount.

Nb is added in accordance with need in the present invention. While depending on the amounts of C, N, and S contained, it forms carbides, nitrides, sulfides, and other fine precipitates in large amounts in steel sheet and causes a remarkable deterioration in the iron loss, promotes the growth of the {111} texture after cold rolling and annealing, and reduces the magnetic flux density, so in the present invention steel does not really have to be added. For this reason, it making the upper limit of Nb 8% or less, preferably 0.02% or less, 0.0030% or less, it becomes possible to obtain good iron loss.

However, carbides and nitrides of Nb (hereinafter in this Description referred to as "Nb precipitates") have the action of retarding the recrystallization of steel sheet, so it is possible to actively use this in the present invention. Further, the fine Nb precipitates also have the effect of increasing the strength in a range not exerting a detrimental effect on the magnetic properties. Further, the Nb can also be utilized as solid solution Nb for strengthening. If present the content of Nb is 0.03 to 8.0% in the present invention. The range may be limited to 0.05 to 8.0%.
The content is preferably 0.08 to 2.0%.

In addition, almost all elements utilized for increasing the strength in high strength electrical steel sheet in the prior art are not only viewed as problems in terms of the costs of addition, but also have some detrimental effect on the magnetic properties, so do not really have to be added. When positively added, from the balance of the recrystallization retardation effect, strength increasing effect, rise in costs, and deterioration of magnetic properties, one or more of Ti, Zr, V, B, Ni, and Cr are added, but the amounts of addition are made Ti: 1.0% or less, Zr: 1.0% or less, V: 1.0% or less, B: 0.010% or less, Ni: 15.0% or less, and Cr: 15.0% or less.

Ti, Zr, and V are elements which form fine precipitates of carbides, nitrides, sulfides, etc. in steel sheet and have the effect of increasing the strength as well, but compared with Nb, the effects are small yet the tendency to cause deterioration of the iron loss is stronger. Further, when forming a partial recrystallized structure in the annealing step after cold rolling, there is a strong effect of promoting alignment in the {111} orientation disadvantageous to improvement of the magnetic flux density, so in the present invention steel, this rather can become harmful elements. For this reason, when not intending strengthening by precipitates, it is preferable to make the contents 1.0% or less. By making the contents preferably 0.50% or less, more preferably 0.30% or less, still more preferably 0.010% or less, further 0.0050% or less, good iron loss can be obtained.

Note that Nb, Zr, Ti, V, and other carbide, nitride, and sulfide forming elements should be prevented from precipitating in the present invention so long as not utilizing the precipitating effects of this as explained above. Nb+Zr+Ti+V is less than 0.1%, preferably less than 0.08%, more preferably 0.002 to 0.05%.

B segregates at the crystal grain boundaries and has the effect of suppressing embrittlement due to grain boundary segregation of P, but in the present invention steel, embrittlement does not become a particular problem like with the conventional mainly solid solution strengthened high strength electrical steel sheet, so addition for this objective is not important. Rather, 0.0002% or more should be added for the purpose of retarding recrystallization due to the effects of the solid solution B on the recrystallization degree. If over 0.010%, remarkable embrittlement occurs, so the upper limit is made 0.010%.

Ni is also recognized as having the effect of raising the recrystallization degree from about 0.001%. Even with a content of 0.01% or less, it has a certain effect in fixing dislocations, but preferably is contained in 0.05%, 0.1%, 0.5%, 1.0%, 2.0%, or further 3.0% whereby its effects are manifested more clearly. Ni further is known to be effective for the prevention of surface defects at the time of hot rolling due to the Cu as an element included in accordance with need in the invention steel (Cu defects). This may also be positively added for this objective as well. Further, it is relatively small in detrimental effects on the magnetic properties and has the effect of improvement of the magnetic flux density and is further recognized as being effective for increasing the strength, so is an element often used in high strength electrical steel sheet. When using Ni for the purpose of preventing Cu defects, it is as a rough standard added in an amount of 1/8 to ½ or so of the amount of Cu.

When utilizing solid solution Cu to increase the strength as explained later, by including Ni compositely, a remarkable effect of reduction of the eddy current loss never seen in the past is exhibited. The reason for this is not clear, but it could be the effect of the positions occupied by the solid solution Cu and solid solution Ni on the Fe crystal lattice and somehow the formation of a regular lattice relating to Ni and Cu.

Further, Ni is also effective for improving the corrosion resistance, but considering the cost of addition and the detrimental effect on the magnetic properties, the upper limit is preferably made 15%, further 10%, still further 5.0%.

Cr is an element added for improving the corrosion resistance and improving the magnetic properties in the high frequency range, but again considering the cost of addition and the detrimental effect on the magnetic properties, the upper limit is made 15.0%.

In particular, when utilizing solid solution Cu as explained later, these roles are sufficiently filled by the Cu (or other elements like Ni), so there is really no need for addition for this purpose. When utilizing solid solution Cu, the Cr is rather added for controlling the stability of the ferrite phase at a high temperature, but the drop in the magnetic flux density due to the addition is remarkable and the element rather can become harmful. Further, the effect of reduction of the eddy current loss due to the solid solution Cu is remarkably expressed in low Cr steel, so unless there is some sort of need, Cr is preferably not added. The reason is not clear, but the effect of the solid solution Cu is believed to become remarkable due to the phenomenon of interaction with not only the above Si, Al, and Ni, but also other elements including Cr. From this viewpoint, considering also the cost of addition, the upper limit of Cr is made 15%, preferably 8.0%, more preferably 4.9%, more preferably 2.9%, more preferably 1.9%, more preferably 0.9%, and more preferably 0.4%.

Further, regarding other trace amount elements, in addition to the amounts unavoidably included from the ore, scraps, etc., even if added in various known ways, the effect of the present invention is not impaired in any way. Further, even if the amounts are small, these are elements forming fine carbides, sulfides, nitrides, oxides, etc. and exhibiting not insignificant recrystallization retardation effects or strength increasing effects, but these fine precipitates also have large detrimental effects on the magnetic properties. Further, in the present invention steel, the residual worked and restored structures enable a sufficient recrystallization retardation effect to be obtained, so these elements need not really be added.

The unavoidable content of these trace amount elements is usually 0.005% or less for each element, but addition of 0.01% or so or more is also possible for various purposes not described in this description. In this case as well, from the balance with the magnetic properties, the one or more types of Bi, Mo, W, Sn, Sb, Mg, Ca, Ce, La, and Co are made a total of 0.5% or less.

The steel including the above ingredients is melted by a converter in the same way as ordinary electrical steel sheet, is continuously cast into a slab, then is hot rolled. The hot rolled sheet is annealed, cold rolled, final annealed, etc. to be produced. Going through steps for formation of an insulating coating or decarburization etc. in addition to these steps does not detract from the effects of the present invention in any way. Further, there is also no problem even if produced not by the usual steps, but by the steps of production of strip by rapid cooling and solidification, the continuous casting of thin slabs without any hot rolling step, etc.

### [Worked Structures]

In the present invention, it is necessary to form special structures called "worked structures" in the present invention in the steel sheet. The "worked structures" in the present invention are differentiated from the "recrystallized structures" accounting for almost the entire steel sheet in ordinary electrical steel sheet. In general, this indicates structures where the strain accumulated in the steel sheet due to cold rolling etc. has not fully disappeared. More specifically, in the process of annealing cold rolled steel sheet, structures deformed by cold rolling and containing a high density of dislocations are encroached upon by structures with a low density of dislocations formed by holding the steel at a high temperature in the annealing step ("recrystallized structures") resulting in progression of recrystallization. The regions not encroached upon by these "recrystallized structures" are defined as the "worked structures". The worked structures generally become lower in density of dislocations due to the so-called restoration etc. during annealing, but do not become as low as the recrystallized structures. In the distribution of strain, there is an uneven state between the "worked structures" and "recrystallized structures". Further, the "worked structures" may be obtained by further working the recrystallized structures. In this case, if viewed overall, the state becomes one where uniform strain remains in the structure. In the present invention, the worked structures are utilized to achieve the targeted higher strength.

### [Grain Size Before Working]

Next, the average crystal grain size d of the steel sheet right before the step of forming the worked structures to finally remain inside the steel sheet characterizing the present invention will be explained. Below, this grain size will be called the "grain size before working". The present invention basically coarsens the "grain size before working" to greatly improve the properties after working, in particular the strength-iron loss balance. The "grain size before working" becomes the grain size at the point of time of the hot rolled sheet when cold rolling the hot rolled sheet, then suppressing recrystallization in the subsequent annealing so as to leave worked structures in the final product. At this time, if annealing the hot rolled sheet as generally performed in electrical steel sheet, the grain size after annealing the hot rolled sheet becomes the "grain size before working". Further, when again cold rolling steel sheet cold rolled, then recrystallized so as to leave worked structures in the final product, this becomes the grain size at the point of time of the annealed sheet. Further, when for example cold rolling the sheet, then again cold rolling it while leaving worked structures in the annealing step, the effect of the working by the repeated cold rolling may be great, but the worked structures formed by the cold rolling will not completely disappear and will remain until after the repeated cold rolling when repeatedly being cold rolled, so the grain size before cold rolling, that is, if the usual steps, the hot rolled sheet grain size, will become the "grain size before working".

In the present invention, this "grain size before working" d (µm) is defined as a specific range in relation to the amount of Si and the amount of Al. That is, by satisfying the following formulae (1), (3) and (4), the superior strength-iron loss balance characteristic of the present invention is achieved: $d \geq 150 μm$ $d \leq \left(400-50\times Si%\right) ,$ and $d \leq \left(820-200\times Si%\right)$

Formula (1) simply shows the case where the "grain size before working" is coarser than a specific size. The crystal grain size of usual steel sheet is controlled to a range of several µm to several hundreds of 100 µm, but to obtain the effect of the present invention, it must be made 20 µm or more. The size is preferably 50 µm or more, more preferably 100 µm or more, more preferably 150 µm or more, more preferably 200 µm or more, more preferably 250 µm or more.

Formula (3) and Formula (4) give rough standards for the upper limit of the "grain size before working". In general, the higher the Si in the material, the brittler the material, but if the "grain size before working" becomes excessively coarse, it becomes further brittle and cold rolling and other working become difficult, so sometimes an upper limit becomes necessary. This upper limit depends not only the steel ingredients other than the amount of Si and the heat history up until working, but also the method of working the steel sheet and the properties aimed at.

The specific conditions for controlling the "grain size before working" to the above range depend also on the steel ingredients and the heat history until working, so cannot be limited to specific ranges, but a person skilled in the art having the usual knowledge would not find it hard to determine suitable conditions by running heat treatment tests several times on steel sheet with the ingredients and heat history corresponding to the targeted steel sheet. To point is to confirm the steel sheet recrystallization and grain growth behavior and just control the heat history so that the aimed at structure is obtained.

As the steel ingredients, raising the purity facilitates formation of coarse grains. In particular, reduction of the C, N, and P is effective. Further, making by ingredients a ferrite single phase steel and suppressing transformation during hot rolling makes coarsening of the grains of the hot rolled sheet easier to achieve.

Further, if oriented at coarser grains in the hot rolled sheet, raising the hot rolling heating temperature, raising the hot rolling finishing temperature, reducing the reduction rate after hot rolling finishing, slow cooling after final rolling, high temperature coiling, high temperature long term hot rolled sheet annealing, etc. may be considered. Further, if oriented at coarser grains in the annealed sheet, high temperature long term annealing is simple, but it is also possible to make the precipitates coarser and improve the grain growth at the time of annealing by low temperature slab heating or high temperature coiling in the hot rolling or high temperature hot rolled sheet annealing conditions. Specifically, for example, it is preferable to make the annealing step right before forming the worked structures any one of the following.
(1) When performing the cold rolling two times or more interspaced with process annealing, performing the process annealing right before the final cold rolling at a temperature of over 850°C (preferably 860°C or more) or for a time over 30 sec (preferably 35 sec or more).
(2) When performing the cold rolling just a single time, when annealing the hot rolled sheet, annealing the hot rolled sheet at a temperature of over 1100°C (preferably 1110°C or more) or for a time over 30 sec (preferably 35 sec or more).
(3) When not the above (1), performing the coiling at the hot rolling at a temperature of over 700°C (preferably 710°C or more).

### [Recrystallization Rate in Structure Before Working]

Note that depending on the conditions, sometimes worked structures remain in the steel sheet right before the step of forming the worked structures to finally remain inside the steel sheet. In this case, to obtain the effect of the present invention, it is preferable not to allow worked structures to remain right before the step of forming the worked structures as much as possible. According to the invention the recrystallization rate r right before the step of forming the worked structures meets $r \geq 50 %$

Preferably, r is 90% or more. Needless to say, right before the step of forming the worked structures, according to the invention a complete recrystallized structure satisfies the above formulas (1) to (4). Further, when not yet recrystallized regions partially remain in the structure right before the step of forming the worked structures, it is possible to obtain the effect of the invention by satisfying the above formula (5), but when the grain size of the recrystallized parts is coarse, even if the not yet recrystallized parts exceed 50%, the effects of present invention will sometimes appear. At this time, by assuming the not yet recrystallized parts are fine crystal grains of a grain size of 5 µm and finding the average grain size, it is possible to judge the effect of the invention by the formula (1). This case is also included in the present invention.

### [Method of Measurement of Grain Size Before Working]

Note that the crystal grain size and recrystallization rate are found by observation of the structure of the sheet cross-section by etching as usually performed in observation of the structure of ferrous metals. The grain size is the diameter found from the area per crystal grain observed when assuming the cross-sectional area of the grain is a circle, while the recrystallization rate is found from the area rate of not yet recrystallized parts in the observed area. Needless to say the measurement has to be performed for a sufficiently average region without segregation.

### [Effect of Grain Size Before Working]

The mechanism for the effect of the "grain size before working" is not certain, but the effects of the change of the dislocation structure, the change of the texture, further the change in the dislocation structure after working due to the difference in texture before working, etc. may be considered. While the details are unclear, it is conjectured that in the end, the dislocation structures in the worked structures change to structures acting as powerful obstructions to dislocations trying to move due to external stress and not easily acting as obstructions to domain walls trying to move due to the external magnetic field.

### [Tensile Strength]

The steel sheet covered by the present invention has a tensile strength of 500 MPa or more. If a steel sheet with a tensile strength of an extent lower than this, even with a steel sheet mainly strengthened by the usual Si, Mn, and other solid solution elements and structurally completely occupied by recrystallized structures, production becomes possible without causing the productivity to deteriorate that much. This is because such a material gives sheet remarkably superior in magnetic properties. The present invention is limited to high strength materials mainly strengthened by the usual solid solution strengthening and unable to be produced without deterioration of the productivity. To enjoy the merits of the present invention more, the invention should be applied to preferably 600 MPa or more steel sheet, more preferably 700 MPa or more, more preferably 800 MPa or more steel sheet. Even production of 900 MPa or more steel sheet not being produced at all at the present is possible. Further, even 1000 MPa or more steel sheet not even imagined for production in the future can be produced with a high productivity.

Note that when used as the rotor of a motor, a slight deformation means the end of the life of the part, so not the tensile strength, but the yield stress should be used for evaluation. The invention steels have worked structures remaining in them, so compared with solid solution strengthened steel or precipitation strengthened steel, if the same strength, the yield stress is higher and, in comparison with these conventional materials, more desirable properties are exhibited. That is, the yield ratio becomes a relatively high value of 0.7 to 1.0 or so. The correlation between the yield stress and the tensile strength becomes extremely strong in the material. For this reason, even if using the yield stress for evaluation, the superiority of the invention steels does not change at all. The effect of the invention is exhibited without problem even for applications like rotors where the yield stress becomes a problem.

### [Area Rate of Worked Structures]

The worked structures are present in an area rate in observation of the cross-sectional structure of steel sheet of 1% or more. The cross-sectional area is observed in the present invention by a cross-section where one side of the cross-section becomes the steel sheet rolling direction and the other side becomes the steel sheet thickness direction. The method performed with ordinary steel sheet of using Nital or another chemical to etch and expose the structure is used, but the invention is not particularly limited in method of observation. Any technique enabling differentiation of the recrystallized structure and the worked structures may be used.

If the area rate of the worked structures is 1% or less, the effect of increasing the strength becomes smaller. When the worked structures are substantially 0%, the result becomes the ordinary steel sheet itself. By controlling the rate to the range of 0 to 1%, the effect of increasing the strength is smaller yet it is necessary to extremely strictly control the temperature of the annealing so this is not practical. To obtain the level of strength actually required, the area rate of the worked structures is controlled to preferably 5% or more, more preferably 10% or more, more preferably 20% or more, more preferably 30% or more, more preferably 50% or more, more preferably 70% or more. There is no problem at all even if made 100% worked structures where substantially no recrystallized structures are observed at all. In this case, the result becomes a so-called "full hard" state which does not anneal at all or the state where annealing is performed, but the structure is restored to the state before the start of recrystallization.

Note that even if the worked structures are less than 95%, 90%, 85%, 80%, or further 75%, the effect of the present invention is obtained.

### [Formation of Worked Structures]

In the steel sheet of the present invention, the structure is adjusted in accordance with the strength and magnetic properties needed, but this adjustment can be performed by the steel ingredients, hot rolling history, cold rolling rate, annealing temperature, annealing time or heating speed, cooling rate, etc. A person skilled in the art can perform this without any problem at all by repeated trials. Alternatively, steel sheet annealed so that the recrystallized structures account for the entire weight may be given strain by repeated cold rolling etc. to form worked structures. In this case, usually the strain is given macroscopically evenly, so the entire amount of the structure becomes worked structures or corresponding to 100% worked structures. In this case, the steel ingredients, heat history, properties, etc. before working are considered and the amount of work is used to control the strength and magnetic properties. This is also possible for a person skilled in the art without problem by several trials.

As a rough standard, with so-called ordinary low grade electrical steel sheet with an amount of Si of 1% or so or less, the temperature is not over 700°C, while even with so-called ordinary high grade electrical steel sheet with an amount of Si of 3% or so, the temperature is not over 800°C or so, but for example by adding suitable amounts of Cu, Nb, etc., it is possible to obtain invention steels of completely restored structures not recrystallizing at all even at a temperature of 900°C or so or more. On the other hand, annealing at a temperature very different from ordinary electrical steel sheet requires a major change in the furnace temperature and not only invites a drop in the work efficiency, but also causes problems in safety as well as mentioned above due to the production of unburned gas. The lower limit of the annealing temperature for avoiding these problems due to extremely low temperature annealing is 400°C or so or more.

The rough standard for the annealing time depends on the temperature as well, but at least 5 seconds or so is required for giving an annealing effect. The annealing time cannot be unambiguously explicitly shown since it depends on the ingredients, production history up to the heat treatment, etc., but the rough standard is, if 850°C, within 5 minutes, if 750°C, within one hour, and, if 600°C, without 10 hours. As explained above, the temperature and time conditions enabling the effect of the invention to be enjoyed can be found without problem by a person skilled in the art by several trials. The point is confirmation of the recrystallization behavior of the steel sheet covered.

When newly forming worked structures by repeated cold rolling etc., if the amount of work is low, it is sometimes difficult to clearly determine the existence of worked structures by the above method of observation of structure, but as a rough standard for sufficiently obtaining the effect of the invention, it is possible to use the (size of crystal grains in sheet thickness direction)/(size of crystal grains in rolling direction) in observation of the cross-sectional structure. This value is made 0.9 or less. If 0.8 or less, the effect of increasing the strength is clearly obtained. The value is preferably 0.7 or less, more preferably 0.6 or less, more preferably 0.5 or less, more preferably 0.3 or less. However, if this value is excessively low, the deterioration of the magnetic properties becomes remarkable, so caution is required.

The above working is usually performed by cold rolling, but there is no need to insist on this so long as there is a change in amount of strain or material quality with the prescription of the present invention. Warm rolling, hot rolling of an extent where the worked structures do not disappear, tensile deformation by imparting tension, bending deformation by a leveler etc., shot blasting, forging, or another method may be used. Rather, due to the method of imparting strain, the dislocation structure is made to change to one preferable for the present invention explained later, so further improvement in properties becomes possible.

In the case of performing this working by cold rolling, the rough standard of the reduction rate can be easily estimated from the ratio of the size of the crystal grains, but is 10 to 70% or so. When further again cold rolling material softened to a certain extent in such an annealing step so as to harden it, the material can easily be made thinner and the productivity of the very thin electrical steel sheet which had been difficult to make in the past is also improved. Such very thin electrical steel sheet according to the present invention enables suppression of the eddy current loss in the case of use under a high frequency magnetic field, so also has the merit of being effective for reduction of the iron loss.

Note that even now there is electrical steel sheet being shipped out after rolling recrystallization annealed steel sheet by 1 to 20% or so skin pass rolling like with the other method of the present invention, that is, so-called semiprocess electrical steel sheet. This skin pass rolled sheet is shipped out as a product, worked by motor manufacturers into motor parts, then annealed under conditions whereby recrystallization will sufficiently occur to cause strain-induced grain growth and thereby obtain a coarse recrystallized structure. This is a means for improving the magnetic properties and is also sometimes called the skin pass method. In this method, no worked structures are ever left at the time of use as a member.

### [Heat Treatment After Formation of Worked Structures]

The present invention inherently differs from this steel sheet and method. It basically does not perform any heat treatment after working the sheet into the part of the electrical equipment. Even when performing some sort of heat treatment by bonding the steel sheet or surface control etc., the worked structures prescribed in the present invention will not disappear and will remain in the range prescribed by the present invention. This is because if the worked structures disappear or deviate from the prescribed range of the present invention, the strength of the steel sheet required in the state of use as an actual motor will become insufficient. The rough standard of the temperature of this heat treatment is the same as the temperature conditions in the above step of annealing the steel sheet. The optimal conditions for enjoying the effect of the invention can be found with the cooperation of persons skilled in the art of production of steel sheet or, even without such cooperation, without any problem by several trials by a usual manufacturer of electrical equipment.

### [Dislocation Density]

The effect of the "worked structures" explained above can also be evaluated by the dislocation density in the "worked structures". The average dislocation density in the worked structures is 1×10¹³/m² or more, more preferably 3×10¹³/m² or more, more preferably 1×10¹⁴/m² or more, more preferably 3×10¹⁴/m² or more. This dislocation density is measured by a transmission type electron microscope. In ordinary electrical steel sheet where the entire amount of the steel sheet is recrystallized structures, the average dislocation density is 1×10¹²/m² or so or less, so is 10 times or more the difference sufficient for discrimination of the worked structures.

Note that strictly speaking, to use even ordinary electrical steel sheet as various members, manufacturers etc. shear, swage, and otherwise work it. Due to this, it is known that some strain remains introduced into the steel sheet and that this has an effect on the properties of the members. This sort of strain is introduced only to the worked locations of the steel sheet and differs from the strain consciously made present at the entire surface of the steel sheet in the present invention, so does not contribute much at all to achieving high strength of the member as a whole.

### [Reason Why Magnetic Properties Can Be Maintained]

The reason why the good magnetic properties can be maintained even if leaving worked structures in the material as in the present invention is not clear, but is believed to be something like the following. In the past, worked structures were considered to cause the magnetic properties to greatly deteriorate and were not regarded as means for achieving high strength of the material. High strength was achieved by refinement of the crystal grains, solid solution strengthening, precipitation strengthening, etc. However, demands for higher strength of materials have been steadily escalating. The conventional means for achieving high strength are now being forced to deal with even regions of conditions remarkably degrading the magnetic properties. When viewing the means for achieving high strength utilizing worked structures once again under such conditions, it appears in some sense that it can no longer be said to be such a disadvantageous method.

Further, what had been conventionally studied was the effect of worked structures in cold rolling of materials where the amount of strain was relatively small in range. Under such conditions, it is believed that the dislocation structures in the material are not relatively even and relatively stable dislocation arrangements like so-called cell structures or restored structures are not formed. Such an extent of working was not attractive at all as means for achieving high strength. Further, with such dislocation structures, the dislocations only became obstructions to domain wall movement. The magnetic properties remarkably deteriorated so this was apparently never practically applied.

On the other hand, when cold working with a relatively high amount of strain like in the present invention or in worked structures restored by annealing, the dislocations form relatively stable cell structures. The cells are normally of a diameter of 1 µm to 0.1 µm or so. Except for the fact that the cell boundaries are formed by dislocations and the difference in crystal orientations with adjacent cells is small, they have structures similar to general crystal grains. They can be viewed as one type of superfine crystal grains and are believed not to easily obstruct domain wall movement. Further, such superfine crystal grains are high in strength and have corresponding ductility when working is required. When considering the balance of strength and magnetic properties, this is believed to be of a level sufficiently enabling practical use. Further, even in the invention steels where worked structures are present, in applications such as use under a high frequency magnetic field where the contribution of the eddy current loss is particularly large in the iron loss, the addition of Si, Mn, Al, Cr, Ni, etc. is important. This has a great effect on the work hardening behavior, the recrystallization behavior, etc., so the development of dislocation strengthened steel based on electrical steel sheet has completely different meaning from that in so-called working use ordinary steel used for automobiles, containers, etc.

### [Applications]

Note that the effects of present invention do not depend on the presence or type of the surface coating formed on the surface of ordinary electrical steel sheet or further on the production steps, so the invention can be applied to nonoriented or grain-oriented electrical steel sheet. In particular, the invention steel can give features very different from steel sheet of conventional recrystallized structures in the in-plane anisotropy of properties. If viewing the magnetic flux density, in the as cold rolled full hard state, the properties of the direction 45° from the coil rolling direction (D direction) are higher than the properties in the rolling direction (L direction) or coil width direction (C direction). Electrical steel sheet having ordinary recrystallized structures in almost all cases have properties in the D direction lower than the properties in the L or C direction. Considering this, by suitably adjusting the extents of the recrystallization and restoration and controlling the structure to the intermediate recrystallization stage, it is possible to easily obtain steel sheet with almost no in-plane anisotropy. Almost no in-plane anisotropy means steel sheet having features enabling extremely preferable properties to be exhibited depending on the applications such as rotary machines.

The applications are not particularly limited. In addition to the applications for rotors of motors used in household electrical appliances, automobiles, etc., the invention may also be applied to all applications where strength and magnetic properties are sought.

### EXAMPLES

### (Example 1)

A slab of 200 mm thickness having the ingredients of 0.002%C-3.0%Si-0.5%Mn-0.03%P-0.001%S-0.3%Al-0.002%N was hot rolled by a slab heating temperature of 1100°C and a coiling temperature of 700°C. The hot rolled sheets were annealed to 800, 950, and 1050°C to change the grain sizes to 10, 100, and 200 µm. These hot rolled sheets were cold rolled, then either not annealed or annealed at 400 to 1000°C for 30 sec to produce product sheets of sheet thicknesses of 0.5 mm differing in recrystallization rate and strength. These were evaluated for mechanical properties using JIS No. 5 test pieces and properties of iron loss W_{10/400} by 55 mm square SST tests. The average values of the mechanical properties and magnetic properties for the coil rolling direction, 45° direction, and direction perpendicular to that were found by the following formula: $X = \left({X}_{0}+2\times {X}_{45}+{X}_{90}\right) / 4$ where, X₀, X₄₅, and X₉₀ are the properties in the coil rolling direction, 45° direction, and direction perpendicular to that.

The results are shown in FIG. 1. As clear from the results, materials with coarse hot rolled sheet grain sizes, that is, materials produced under the conditions of the present invention, are excellent in strength-iron loss balance.

**Table 1**

| No | Ingredients (mass%) | | | | | | | | | |
|---|---|---|---|---|---|---|---|---|---|---|
| | C | Si | Mn | P | S | Al | N | Cu | Nb | Others |
| | | | | | | | | | | |
| 2 | 0.0010 | 3.0 | 0.8 | 0.010 | 0.0005 | 1.64 | 0.0019 | - | - | - |
| 3 | 0.0010 | 3.0 | 0.8 | 0.010 | 0.0005 | 1.64 | 0.0019 | - | - | - |
| 4 | 0.0025 | 0.7 | 0.21 | 0.090 | 0.0025 | 0.001 | 0.0024 | - | - | - |
| 5 | 0.0025 | 0.7 | 0.21 | 0.090 | 0.0025 | 0.001 | 0.0024 | | - | - |
| 6 | 0.0025 | 0.7 | 0.21 | 0.090 | 0.0025 | 0.001 | 0.0024 | - | - | - |
| 7 | 0.0025 | 0.7 | 0.21 | 0.090 | 0.0025 | 0.001 | 0.0024 | - | - | - |
| 8 | 0.0019 | 2.1 | 0.20 | 0.060 | 0.0012 | 0.22 | 0.0026 | - | - | - |
| | | | | | | | | | | |
| | | | | | | | | | | |
| | | | | | | | | | | |
| 12 | 0.0012 | 2.9 | 0.40 | 0.030 | 0.0005 | 0.5 | 0.0013 | 3.9 | - | Ni: 1.8 |
| 13 | 0.0012 | 2.9 | 0.40 | 0.030 | 0.0005 | 0.5 | 0.0013 | 3.9 | - | Ni: 1.8 |
| 14 | 0.0006 | 3.1 | 0.30 | 0.008 | 0.0009 | 0.15 | 0.0025 | - | - | Ni: 2.0 Cr: 5.0 |
| 15 | 0.0230 | 2.5 | 1.20 | 0.022 | 0.0006 | 0.06 | 0.0036 | - | 0.11 | B: 0.008 |
| 16 | 0.0230 | 2.5 | 1.20 | 0.022 | 0.0006 | 0.06 | 0.0036 | - | 0.11 | B: 0.008 |
| 17 * | 0.0008 | 3.4 | 0.53 | 0.041 | 0.0004 | 0.02 | 0.0024 | - | 0.37 | Ti: 0.35 |
| 18 * | 0.0008 | 3.4 | 0.53 | 0.041 | 0.0004 | 0.02 | 0.0024 | - | 0.37 | Ti: 0.35 |
| 19 | 0.0322 | 3.1 | 0.50 | 0.016 | 0.0002 | 1.2 | 0.0011 | - | 1.3 | - |
| 20 | 0.0322 | 3.1 | 0.50 | 0.016 | 0.0002 | 1.2 | 0.0011 | - | 1.3 | - |
| 21 | 0.0077 | 2.9 | 0.29 | 0.023 | 0.0015 | 0.8 | 0.0022 | 2.1 | - | - |
| 22 * | 0.0021 | 3.7 | 0.05 | 0.002 | 0.0009 | 0.24 | 0.0026 | - | - | Sn: 0.09 Ce: 0.002 |

| | | | | | | | | | | |
|---|---|---|---|---|---|---|---|---|---|---|
| (Balance of Fe and unavoidable impurities) * not within the claims | | | | | | | | | | |

### (Example 2)

From slabs of 200 mm thickness having the ingredients of Table 1, product sheets were produced under the production conditions shown in Table 2. Some of the materials were heat treated assuming the heat treatment at motor manufacturers (user annealing). These were evaluated for mechanical properties using JIS No. 5 test pieces and properties of iron loss W_{10/400} and magnetic flux density B₂₅ by 55 mm square SST tests. The average values of the mechanical properties and magnetic properties for the coil rolling direction, 45° direction, and direction perpendicular to that were found by the following formula: $X = \left({X}_{0}+2\times {X}_{45}+{X}_{90}\right) / 4$ where, X₀, X₄₅, and X₉₀ are the properties in the coil rolling direction, 45° direction, and direction perpendicular to that.

The results are shown in Table 2. As clear from the results, materials produced under the conditions of the present invention are hard and further superior in magnetic properties. Caution is required in that generally electrical steel sheet greatly differ in properties due to the amount of Si so are graded and sold according to the amount of Si contained. Further, the iron loss greatly changes depending on the sheet thickness. A high Si material, compared with a low Si material, greatly drops in iron loss due to the difference in Si content. Further, even sheets with thin sheet thicknesses fall in iron loss, so when evaluating the effect of the present invention, it is necessary to bear in mind the differences in the amounts of Si and sheet thicknesses and compare sheets with equivalent amounts of Si and sheet thicknesses.

### INDUSTRIAL APPLICABILITY

According to the present invention, it is possible to stably produce hard high strength electrical steel sheet superior in magnetic properties. That is, the present invention enables the targeted strength to be obtained even with relatively low amounts of the added elements used for solid solution strengthening and precipitation strengthening, so the cold rollability is improved, the productivity of the cold rolling step is improved, and annealing in the usual operating range becomes possible, so the work efficiency in the annealing step also is improved. Further, by cold rolling again after annealing, it becomes possible to simply produce extremely thin materials which were difficult to produce in the past.

From the above, the strength, fatigue strength, and wear resistance can be secured, so increased efficiency, smaller size, longer lifetime, etc. of superhigh speed motors, motors with magnets built into the rotors, and materials for electromagnetic switches are achieved.

## Claims

1. A method of production of high strength electrical steel sheet containing, by mass%, C: 0.060% or less, Si: 0.2 to 3.2%, Mn: 0.05 to 3.0%, P: 0.30% or less, S or Se: 0.040% or less, Al: 2.50% or less, and N: 0.040% or less, optionally further containing by mass%, one or both of Cu: 0.001 to 30.0% and Nb: 0.03 to 8.0%; optionally further containing by mass%, one or more types of Ti: 1.0% or less, V: 1.0% or less, Zr: 1.0% or less, B: 0.010% or less, Ni: 15.0% or less, and Cr: 15.0% or less; and optionally further containing by mass%, one or more types of Bi, Mo, W, Sn, Sb, Mg, Ca, Ce, La, and Co in a total of 0.5% or less; having a balance of Fe and unavoidable impurities, and having worked structures not encroached upon by recrystallized structures remaining inside the steel sheet, said method of production of high strength electrical steel sheet being **characterized by** making an average crystal grain size d of the steel sheet right before the final cold rolling step 150 µm or more, making
d≤(400-50xSi%) and
d≤(820-200xSi%),
and
making the recrystallization rate of the steel sheet right before the step of forming the worked structures to finally remain inside the steel sheet 50% or more.

2. The method of production of high strength electrical steel sheet as set forth in claim 1 **characterized in that** the steel ingredients contain, by mass%, one or both of Cu: 0.001 to 30.0% and Nb: 0.03 to 8.0%.

3. The method of production of high strength electrical steel sheet as set forth in any one of claims 1 to 2 **characterized in that** the steel ingredients contain, by mass%, one or more types of Ti: 1.0% or less, V: 1.0% or less, Zr: 1.0% or less, B: 0.010% or less, Ni: 15.0% or less, and Cr: 15.0% or less.

4. The method of production of high strength electrical steel sheet as set forth in any one of claims 1 to 3 **characterized in that** the steel ingredients contain, by mass%, one or more types of Bi, Mo, W, Sn, Sb, Mg, Ca, Ce, La, and Co in a total of 0.5% or less.

5. The method of production of high strength electrical steel sheet as set forth in any one of claims 1 to 4 **characterized in that** the worked structures present inside the steel sheet are 1% or more by area rate in observation of the cross-section.

6. The method of production of high strength electrical steel sheet as set forth in any one of claims 1 to 5, **characterized in that** an average dislocation density in the worked structures inside the steel sheet is 1x10¹³/m² or more.

## Patentansprüche

1. Ein Verfahren zur Herstellung eines hochfesten Elektrostahlblechs, enthaltend, in Massen-%, C: 0,060% oder weniger, Si: 0,2 bis 3,2%, Mn: 0,05 bis 3,0%, P: 0,30% oder weniger, S oder Se: 0,040% oder weniger, Al: 2,50% oder weniger und N: 0,040% oder weniger, gegebenenfalls ferner enthaltend, in Massen-%, eines oder beide von Cu: 0,001 bis 30,0% und Nb: 0,03 bis 8,0%; gegebenenfalls ferner enthalten, in Massen-%, eine oder mehrere Arten von Ti: 1,0% oder weniger, V: 1,0% oder weniger, Zr: 1,0% oder weniger, B: 0,010% oder weniger, Ni: 15,0% oder weniger und Cr: 15,0% oder weniger; und gegebenenfalls ferner enthaltend, in Massen-%, eine oder mehrere Arten von Bi, Mo, W, Sn, Sb, Mg, Ca, Ce, La und Co in einer Gesamtmenge von 0,5% oder weniger; mit einem Rest aus Fe und unvermeidbaren Verunreinigungen; und mit nicht durch rekristallisierte Strukturen beeinträchtigten bearbeiteten Strukturen, die im Inneren des Stahlblechs verbleiben; wobei das Verfahren zur Herstellung eines hochfesten Elektrostahlblechs **dadurch gekennzeichnet ist, dass** eine mittlere Kristallkorngröße d des Stahlblechs unmittelbar vor dem letzten Kaltwalzschritt 150 µm oder mehr beträgt,
d≤(400-50xSi%) und
d≤(820-200xSi%) beträgt,
und
die Rekristallisierungsrate des Stahlblechs unmittelbar vor dem Schritt des Formens der bearbeiteten Strukturen, die abschließend im Inneren des Stahlblechs verbleiben, 50% oder mehr beträgt.

2. Das Verfahren zur Herstellung eines hochfesten Elektrostahlblechs nach Anspruch 1, **dadurch gekennzeichnet, dass** die Stahlbestandteile, in Massen-%, eines oder beide von Cu: 0,001 bis 30,0% und Nb: 0,03 bis 8,0% enthalten.

3. Das Verfahren zur Herstellung eines hochfesten Elektrostahlblechs nach einem der Ansprüche 1 bis 2, **dadurch gekennzeichnet, dass** die Stahlbestandteile, in Massen-%, eine oder mehrere Arten von Ti: 1,0% oder weniger, V: 1,0% oder weniger, Zr: 1,0% oder weniger, B: 0,010% oder weniger, Ni: 15,0% oder weniger und Cr: 15,0% oder weniger enthalten.

4. Das Verfahren zur Herstellung eines hochfesten Elektrostahlblechs nach einem der Ansprüche 1 bis 3, **dadurch gekennzeichnet, dass** die Stahlbestandteile, in Massen-%, eine oder mehrere Arten von Bi, Mo, W, Sn, Sb, Mg, Ca, Ce, La und Co in einer Gesamtmenge von 0,5% oder weniger enthalten.

5. Das Verfahren zur Herstellung eines hochfesten Elektrostahlblechs nach einem der Ansprüche 1 bis 4, **dadurch gekennzeichnet, dass** die bearbeiteten Strukturen, die im Inneren des Stahlblechs vorhanden sind, bei Betrachtung des Querschnitts einen Flächenanteil von 1% oder mehr aufweisen.

6. Das Verfahren zur Herstellung eines hochfesten Elektrostahlblechs nach einem der Ansprüche 1 bis 5, **dadurch gekennzeichnet, dass** eine durchschnittliche Versetzungsdichte in den bearbeiteten Strukturen innerhalb des Stahlblechs 1x10¹³/m² oder mehr beträgt.

## Revendications

1. Procédé de production de tôle d'acier électrique de résistance élevée contenant, en % en masse : C : 0,060 % ou inférieur, Si : 0,2 à 3,2 %, Mn : 0,05 à 3,0 %, P : 0,30 % ou inférieur, S ou Se : 0,040 % ou inférieur, Al : 2,50 % ou inférieur, et N : 0,040 % ou inférieur, éventuellement contenant de plus en % en masse, un ou les deux de Cu : 0,001 à 30,0 % et Nb : 0,03 à 8,0 % ; éventuellement contenant de plus en % en masse, un ou plusieurs types de Ti : 1,0 % ou inférieur, V : 1,0 % ou inférieur, Zr : 1,0 % ou inférieur, B : 0,010 % ou inférieur, Ni : 15,0 % ou inférieur, et Cr : 15,0 % ou inférieur ; et éventuellement contenant de plus en % en masse, un ou plusieurs types de Bi, Mo, W, Sn, Sb, Mg, Ca, Ce, La, et Co dans un total de 0,5 % ou inférieur ; ayant un reste de Fe et impuretés inévitables, et ayant des structures usinées non empiétées par des structures recristallisées restant à l'intérieur de la tôle d'acier, ledit procédé de production de tôle d'acier électrique de résistance élevée étant **caractérisé par** la constitution d'une taille moyenne de grain de cristal d de la tôle d'acier juste avant l'étape de laminage à froid finale de 150 µm ou supérieure, réalisant
d≤(400-50xSi%) et
d≤ (820-200xSi%),
et
faisant que la vitesse de recristallisation de la tôle d'acier juste avant l'étape de formation des structures usinées reste finalement à l'intérieur de la tôle d'acier supérieure ou égale à 50 %.

2. Procédé de production de tôle d'acier électrique de résistance élevée selon la revendication 1, **caractérisé en ce que** les ingrédients d'acier contiennent, en % en masse, un ou les deux de Cu : 0,001 à 30,0 % et Nb : 0,03 à 8,0 %.

3. Procédé de production de tôle d'acier électrique de résistance élevée selon l'une quelconque des revendications 1 à 2, **caractérisé en ce que** les ingrédients d'acier contiennent, en % en masse, un ou plusieurs types de Ti : 1,0 % ou inférieur, V : 1,0 % ou inférieur, Zr : 1,0 % ou inférieur, B : 0,010 % ou inférieur, Ni : 15,0 % ou inférieur, et Cr : 15,0 % ou inférieur.

4. Procédé de production de tôle d'acier électrique de résistance élevée selon l'une quelconque des revendications 1 à 3, **caractérisé en ce que** les ingrédients d'acier contiennent, en % en masse, un ou plusieurs types de Bi, Mo, W, Sn, Sb, Mg, Ca, Ce, La et Co dans un total de 0,5 % ou inférieur.

5. Procédé de production de tôle d'acier électrique de résistance élevée selon l'une quelconque des revendications 1 à 4, **caractérisé en ce que** les structures usinées présentes à l'intérieur de la tôle d'acier sont de 1 % ou supérieures par taux de surface dans une observation de la section transversale.

6. Procédé de production de tôle d'acier électrique de résistance élevée selon l'une quelconque des revendications 1 à 5, **caractérisé en ce qu'**une densité moyenne de dislocation dans les structures usinées à l'intérieur de la tôle d'acier est de 1x10¹³/m² ou supérieure.
